

## UNITED STATES PATENT OFFICE

LEO P. CURTIN, OF CRANBURY, NEW JERSEY

METHOD OF CONVERTING ROASTED LEAD ORES AND BAG-HOUSE DUST DIRECTLY  
INTO LEAD SALTS

No Drawing.

Application filed May 3, 1932. Serial No. 609,044.

In my pending application, Serial No. 570,773, filed October 23, 1931, I have described a method of converting lead ores directly into lead salts without the intermediate formation of metallic lead which consists essentially in treating a roasted galena ore or similar mixture of lead oxide, lead sulfate, and basic lead sulfate, with or without gangue matter, first with a solution of lead acetate to dissolve the basic lead or lead oxide content, and second, with a solution of calcium acetate or ammonium acetate to dissolve the lead sulfate content.

The present invention relates to an improved method of treating such mixtures containing lead oxide, lead sulfate and basic lead sulfate, and is particularly designed and suitable for the treatment of bag-house fume or bag-house dust for converting its lead content directly into valuable compounds without at any point in the process producing metallic lead. The invention will be described and illustrated in connection with the treatment of lead fume, but, as will be apparent, is not limited thereto.

In the smelting of ores it commonly occurs that a small portion of the lead, say 1 to 4%, is volatilized by the heat of the smelting operation and is condensed and collected as fume in what are known as bag-houses. The coarser portions of the fume are called bag-house dust and the finer portions bag-house fume. The composition of this dust and fume varies somewhat at different smelters, but in all cases lead sulfate is a very important constituent and lead in other forms, such as lead oxide or basic lead sulfate, is generally present in substantial quantities. An analysis of the fume from a large smelter in the St. Louis district shows that it contains about 65% of lead calculated as lead metal, and that 77% of this lead is present as sulfate and 23% in basic form. Analyses of the by-product from other smelters may show a somewhat higher percentage of impurities, and also moderate variations in the ratio of basic lead to lead sulfate.

A characteristic of all bag-house sublimates is that they are very largely free from the non-volatile impurities present in

the original ore, such as alumina, silica and various silicates. Substances other than lead compounds which are present in the fume are mainly small amounts of cadmium, zinc, bismuth, antimony and arsenic compounds. As will be seen, the fume is a much purer and more desirable material to use as a raw material than any lead ore, even when such lead ore has been roasted so that its lead is present as oxide, basic sulfate and sulfate.

In the extraction of lead from fume, lead acetate solution alone is valueless because of its inability to dissolve more than traces of lead sulfate. Calcium acetate is a better solvent for the lead sulfate, but has the disadvantage of becoming saturated with soluble lead compounds when the solution contains only two or three per cent of such lead compounds, and furthermore calcium acetate is completely unable to dissolve the more refractory portions of the fume. Sodium acetate is even less effective than calcium acetate and potassium acetate is valueless for the purpose, since it forms an insoluble double sulfate with lead.

It is well known that ammonium acetate is a solvent for lead sulfate and even shows some solvent effects on basic lead sulfate. Its principal disadvantage is that, as ordinarily used, it does not dissolve sufficient lead sulfate to be commercially advantageous, and by bringing the sulfate ion into solution along with the lead, it gives a solution from which it is very difficult to prevent the precipitation of lead as sulfate during subsequent operations with the solution. I have found that, if soluble alkaline earth metal salt, such as an alkaline earth metal acetate, be dissolved in the ammonium acetate solution, in the proper proportion, greatly increased dissolving of the lead content of the fume is obtained, and most of the sulfate is left in the residue as alkaline earth metal sulfate. Furthermore, by utilizing the principles of counter-current washing, it is possible to extract practically all of lead present, leaving a residue of the impurities originally present in the fume, together with crystalline alkaline earth metal sulfate. This residue may be readily separated by

mechanical or chemical means, into alkaline earth metal sulfate, on the one hand, and the cadmium and other compounds previously mentioned, on the other hand, these latter being then worked up in any known manner for other valuable derivatives.

As an alkaline earth metal salt to reinforce the ammonium acetate, I prefer to use calcium acetate because of its cheapness. Other 10 calcium salts may be used, even calcium hydroxid, which may be dissolved in the ammonium acetate or mixed dry with the fume before extraction. In any event, it is desirable to have the solution or the dry fume 15 contain enough calcium salt to convert all of the sulfate present into gypsum.

The advantage of using the calcium salt is that it converts the sulfate present in the fume into an insoluble compound which 20 remains behind in the residue. The resulting solution, under these conditions, contains lead in abundance, but only a small quantity of sulfate ion, and the tendency of lead to precipitate as lead sulfate is, therefore, very 25 greatly reduced. Careful experimentation on different materials has shown that it is possible to dissolve 2½ times as much lead from fume by the use of ammonium acetate in conjunction with calcium acetate as would 30 be obtained if only ammonium acetate were used.

I prefer to use a solution of ammonium acetate ranging from 25 to 35% in concentration and containing as much calcium acetate as experience shows is required to completely react with the sulfate ion present. For example, 100 cc. of a 30% solution of ammonium acetate, containing 5% by weight of calcium ion as either acetate or 35 hydroxid, is capable of dissolving from fume or from lead sulfate as much as 20 grams of lead calculated as metallic lead. As stated above, the proportion of calcium ion may be varied slightly, as experience will 40 indicate. The ammonium acetate solution may be used with good results under neutral, basic, or acid conditions. I find it most convenient to use when it contains a small excess of free acid.

50 The ammonium acetate solution is preferably used hot, temperatures ranging from 90 to 100° C. After dissolving the lead, it is readily separated from the residue by filtration or decantation. The clear filtrate, which 55 is usually water white in color, may then be used to prepare lead salts.

In the preparation of lead chromate or lead arsenate, a soluble chromate or arsenate is added to the lead solution under appropriate conditions. An immediate precipitation of the desired product occurs. In the preparation of white lead or lead basic carbonate it is usually necessary to make the solution 60 alkaline either by using lime in some way in the original extraction or by adding lime or

other alkali to the lead-containing ammonium acetate solution. This solution readily dissolves calcium hydroxide and in so doing regenerates the calcium acetate which is used in the original extracting solution. Carbon 70 dioxide is then introduced into the solution, and lead basic carbonate is thrown down. The precipitate is then filtered out and the solution is now in condition for a second extraction of fume.

The presence of ammonium salts in a lead containing solution from which lead basic carbonate is to be precipitated is of great advantage. When alkali, such as sodium hydroxide or calcium hydroxide, is added to 80 such a solution, the pH of the solution does not increase nearly as much as if the ammonium salts were absent. A great deal of the added base is transformed into ammonium hydroxide by interaction with ammonium 85 acetate, thereby replacing a strong base by a much weaker one. At the concentrations used, ammonium hydroxide is only 1/80 as strong as the corresponding quantity of calcium hydroxide and 1/200 as strong as the 90 equivalent of sodium hydroxide. This holds the pH within a range favorable for the precipitation of lead basic carbonate, while, in the absence of ammonium salts, the solution becomes so basic that the resultant precipitate of lead is more basic than is desirable. 95

I claim:

1. Method of recovering the lead content of material containing lead sulfate which comprises subjecting the material to the solvent action of a solution of ammonium acetate in the presence of a soluble alkaline earth metal compound.

2. Method as defined in claim 1 in which the lead sulfate-containing material contains 105 also lead oxid and lead basic sulfate.

3. Method as defined in claim 1 in which the lead sulfate-containing material is lead fume.

4. Method as defined in claim 1 in which 110 the alkaline earth metal compound is calcium acetate.

5. Method as defined in claim 1 in which the ammonium acetate solution is acidified.

6. Method as defined in claim 1 in which 115 the lead sulfate-containing material is extracted with a solution containing ammonium acetate and a soluble alkaline earth metal compound.

7. Method as defined in claim 1 in which 120 the alkaline earth metal compound is present in quantity sufficient to react with all of the sulfate present in the lead sulfate-containing material to the formation of an insoluble alkaline earth metal sulfate.

8. Method as defined in claim 1 in which the lead sulfate-containing material is treated with ammonium acetate solution by countercurrent washing.

9. Method as defined in claim 1 in which 130

the lead sulfate-containing material is subjected to the solvent action of an ammonium acetate-containing solution at elevated temperature.

5 10. Method of recovering lead from lead fume which comprises extracting the fume with a solution of ammonium acetate and calcium acetate, separating the resulting solu-

tion, adding calcium hydroxid to the solution, treating the solution with carbon dioxide to precipitate its lead content, and using the resulting solution for extracting more lead fume.

In testimony whereof, I affix my signature.

LEO P. CURTIN.

10

75

15

80

20

85

25

90

30

95

35

100

40

105

45

110

50

115

55

120

60

125

65

130